

## UNITED STATES PATENT OFFICE.

WILLIS F. WASHBURN, OF ST. LOUIS, MISSOURI, ASSIGNOR TO NATIONAL PIGMENTS & CHEMICAL COMPANY, OF ST. LOUIS, MISSOURI, A CORPORATION OF MISSOURI.

## METHOD OF BLEACHING BARYTES.

No Drawing.

Application filed April 28, 1924. Serial No. 709,692.

To all whom it may concern:

Be it known that I, WILLIS F. WASHBURN, a citizen of the United States, and residing at St. Louis, State of Missouri, have invented 5 the new and useful Improvement in Methods of Bleaching Barytes, of which the following is a specification.

This invention relates to the art of bleaching barytes, and more particularly to render 10 it suitable for use in the paint, rubber, color and allied industries.

In the art of bleaching barytes as heretofore practiced, the crude material is crushed to suitable size and washed until free from 15 clay and other adhering impurities. It is then placed in suitable mills, usually of the ball or tube type and reduced to the desired fineness. The fine material is then placed in a suitable container and acid (usually sul- 20 phuric acid) added and the mixture is boiled until a sample shows that the desired degree of bleaching has been attained. The action of the acid is to leach out the impurities which are usually present in the form of 25 oxides of iron, manganese, etc., some of which are difficultly soluble in acid, and some of which may not be completely soluble. The time required is, therefore, not only extended and not only is the amount of acid required 30 considerable, but the result may not be a product of the desired color.

One of the objects of this invention, therefore, is to develop a method or process of bleaching in which the time required is not 35 only reduced but in which the resulting product is of a superior color.

Further objects will appear from the detail description in which an embodiment of this invention will be described; it will, however, 40 be understood that the invention may be exemplified in other embodiments.

I have discovered that if a reducing agent is present in the mixture during the bleach, much less time is required for the operation 45 and that the resulting product is of superior color. There are many reducing agents which may be used for this purpose, for example, stannous and titanous salts, the metals which react with acid with liberation of hy- 50 drogen, electrolysis, etc.: an agent especially suitable and convenient for this purpose is metallic iron.

Generally stated in accordance with this invention the barytes is treated with a suitable acid in the presence of a reducing agent,

such as hydrogen. This hydrogen is preferably liberated by the action of an agent, such as described. Where a metal is used, it is preferably such that its salt is soluble; and where iron is used, it is preferably one 60 which is low in carbon, such as wrought iron. The acid used is preferably sulphuric acid, although other acids, such as hydro-chloric acid may be used.

As a practical embodiment of this invention, the process or method may be carried out as follows: Crude barytes is crushed to about 1 inch mesh, washed with water and wet ground in a tube mill to a suitable fineness, such as 250 mesh, and water floated to 70 eliminate any coarse particles. The resulting finely divided barytes, usually in the form of a slurry containing 10 to 25 percent water is pumped into a suitable tank and sulphuric acid added. The amount of acid used may 75 be varied considerably, from 1 to 4 tons 60° Be. acid to 30 tons of slurry has been found to be satisfactory. There is then introduced into the treating tank a suitable quantity of metallic iron, such as wrought iron, which 80 for convenience may be in the form of bars. The amount of iron required depends upon the impurities originally present in the barytes and may be readily determined by trial. The mixture is then boiled by the injection of live steam until the barytes is 85 of the desired color. The bleached barytes is then washed and dried.

As a result of the improved method or process, not only is the resulting product of 90 a superior color, but much less time is required for the operation in order to secure that result. The action is probably due to the reduction of the difficultly soluble or insoluble oxides or other impurities to the more 95 soluble form. It is to be understood, however, that while a theory of operation has been advanced, it is not the only or necessary one but has only been advanced to facilitate the disclosure. It is understood, however, 100 that this invention is not limited to any theory of operation or action. It is further obvious that various changes may be made in details without departing from the spirit of this invention; it is, therefore, to be understood that this invention is not to be limited to the specific details described.

Having thus described the invention, what is claimed is:

1. A method of bleaching barytes consist-

ing in treating the barytes with a mineral acid in the presence of a gaseous reducing agent.

2. A method of bleaching barytes consisting in treating the barytes with a mineral acid in the presence of hydrogen.

3. A method of bleaching barytes consisting in treating the barytes with a mineral acid in the presence of an agent which reacts with the acid with liberation of hydrogen.

4. A method of bleaching barytes consisting in treating the barytes with a mineral acid in the presence of a metal which reacts with the acid with liberation of hydrogen.

5. A method of bleaching barytes consisting in treating the barytes with a mineral acid in the presence of a metal whose salt is soluble.

6. A method of bleaching barytes consisting in treating the barytes with a mineral acid in the presence of metallic iron.

7. A method of bleaching barytes consisting in treating the barytes with sulphuric acid in the presence of low carbon iron.

In testimony whereof I affix my signature this 5th day of April, 1924.

WILLIS F. WASHBURN.